# EUROPEAN PATENT SPECIFICATION

(11) **EP 0 757 725 B1**
(45) Date of publication and mention of the grant of the patent: **08.09.1999**
(21) Application number: 95915455.0
(22) Date of filing: 07.04.1995
(51) Int. Cl.: C23C 22/23, C23C 22/68

(54) **COMPOSITION AND PROCESS FOR TREATING THE SURFACE OF ALUMINIFEROUS METALS**
ZUSAMMENSETZUNG UND VERFAHREN ZUR OBERFLÄCHENBEHANDLUNG ALUMINIUMHALTIGER METALLE
COMPOSITION ET PROCEDE POUR TRAITER LA SURFACE DE METAUX ALUMINEUX

(30) Priority: 15.04.1994 JP 7721994
(43) Date of publication of application: 12.02.1997
(73) Proprietor: HENKEL CORPORATION, Plymouth Meeting, PA 19462 (US)
(72) Inventor: AOKI, Tomoyuki, Chigasaki-shi, Kanagawa-ken 253 (JP); YOSHIDA, Masayuki, Nihon Parkerizing Co., Housing, Yokohama-shi, Kanagawa-ken 241 (JP)
(74) Representative: Sanderson, Laurence Andrew
(86) International application number: US9503933
(87) International publication number: WO9528509

(56) References cited:
- WO-A-91/10756
- AU-B- 647 498
- GB-A- 2 250 025
- US-A- 4 517 028
- US-A- 4 795 506

## Description

This invention relates to a novel composition and method for treating the surface of aluminiferous metals in order thereby to provide such surfaces, prior to their being painted, with an excellent corrosion resistance and paint adherence. This invention may be effectively applied, *inter alia,* to the surface treatment of drawn-and-ironed (hereinafter usually abbreviated "Dl") aluminum cans. When applied to the Dl aluminum cans fabricated by the drawing-and-ironing of aluminum alloy sheet, the surface treatment composition and method according to the present invention are particularly effective in providing the surface of such cans, prior to the painting or printing thereof, with an excellent corrosion resistance and paint adherence and also with the excellent slideability required for smooth conveyor transport of the can (abbreviated below simply as "slideability").

Liquid compositions, which hereinafter are often called "baths" for brevity, even though they may be used by spraying or other methods of establishing contact than immersion, that are useful for treating the surface of aluminiferous metals, defined as aluminum and its alloys that contain at least 45% by weight of aluminum, may be broadly classified into chromate-type treatment baths and non-chromate-type treatment baths. The chromate-type surface treatment baths typically are divided into chromic acid chromate conversion treatment baths and phosphoric acid chromate conversion treatment baths. Chromic acid chromate conversion treatment baths were first used in about 1950 and are still in wide use at present for the surface treatment of, for example, heat exchanger fins and the like. Chromic acid chromate conversion treatment baths contain chromic acid (CrO₃) and hydrofluoric acid (HF) as their essential components and may also contain a conversion accelerator. These baths form a coating that contains small amounts of hexavalent chromium. The phosphoric acid chromate conversion treatment bath was invented in 1945 (see U.S. Patent 2,438,877). This conversion treatment bath contains chromic acid (CrO₃), phosphoric acid (H₃PO₄), and hydrofluoric acid (HF) as its essential components. The main component in the coating produced by this bath is hydrated chromium phosphate (CrPO₄ •4 H₂O). Since this conversion coating does not contain hexavalent chromium, this bath is still in wide use at present as, for example, a paint undercoat treatment for the lid and body of beverage cans.

The treatment bath taught in Japanese Patent Application Laid Open [Kokai or Unexamined] Number Sho 52-131937 [131,937/1977] is typical of the non-chromate-type conversion treatment baths. This treatment bath is an acidic (pH = approximately 1.0 to 4.0) waterborne coating solution that contains phosphate, fluoride, and zirconium or titanium or their compounds. Treatment of aluminiferous metal surfaces with this non-chromate-type conversion treatment bath produces thereon a conversion film whose main component is zirconium and/or titanium oxide. The absence of hexavalent chromium is one advantage associated with the non-chromate-type conversion treatment baths; however, the conversion coatings produced by them in many instances exhibit a corrosion resistance and paint adherence that is inferior to those of the coatings generated by chromate-type conversion treatment baths. Moreover, both chromate-type and non-chromate-type conversion treatment baths contain fluorine, which conflicts with the contemporary desire, prompted by environmental concerns, for the practical implementation of fluorine-free surface treatment baths.

The use of water-soluble resins in surface treatment baths and methods intended to provide aluminiferous metals with corrosion resistance and paint adherence is described, for example, in Japanese Patent Application Laid Open [Kokai or Unexamined] Numbers Sho 61-91369 [91,369/1986] and Hei 1-172406 [172,406/1989], Hei 1-177379 [177,379/1989], Hei 1-177380 [177,380/1989], Hei 2-608 [608/1990], and Hei 2-609 [609/1990]. In these examples of the prior art surface treatment baths and methods, the metal surface is treated with a solution containing a derivative of a polyhydric phenol compound. However, the formation of an acceptably stable resin-containing coating on the aluminiferous metal surface sometimes is highly problematic with these prior art methods, and they do not always provide an acceptable performance (corrosion resistance). The invention described in Japanese Patent Application Laid Open [Kokai or Unexamined] Number Hei 4-66671 [66,671/1992] constitutes an improvement to treatment methods that use polyhydric phenol derivatives, but even in this case the problem of an unsatisfactory adherence sometimes arises.

The surface of Dl aluminum cans is at present treated mainly with the above-described phosphoric acid chromate surface treatment baths and zirconium-containing non-chromate surface treatment baths. The outside bottom surface of Dl aluminum cans is not painted, but is subjected to high-temperature sterilization. If its corrosion resistance is poor, the aluminum will become oxidized at this point and a blackening discoloration will occur, a phenomenon which is generally known as "blackening". In order to prevent blackening, the coating produced by surface treatment must itself, even when unpainted, exhibit a high corrosion resistance.

Tuming to another issue, a high friction coefficient for the can's exterior surface will cause the can surface to have a poor slideability during the conveyor transport that occurs in the can fabrication and finishing processes. This will cause the can to tip over, which will obstruct the transport process. Can transportability is a particular concern with regard to transport to the printer. Thus, there is demand in the can fabrication industry for a lowering of the static friction coefficient of the can's exterior surface, which, however, must be achieved without adversely affecting the adherence of the paint or ink which will be coated on the can. The invention disclosed in Japanese Patent Application Laid Open [Kokai or Unexamined] Number Sho 64-85292 [85,292/1989] is an example of a method directed to improving this slideability. This invention relates to a surface treatment agent for metal cans, wherein said surface treatment agent contains water-soluble organic substance selected from phosphate esters, alcohols, monovalent and polyvalent fatty acids, fatty acid derivatives, and mixtures of the preceding. While this method does serve to increase the slideability of aluminum cans, it affords no improvement in corrosion resistance or paint adherence.

The invention described in Japanese Patent Application Laid Open [Kokai or Unexamined] Number Hei 5-239434 [239,434/1993] is another method directed to improving the slideability of aluminum cans. This invention is characterized by the use of phosphate esters. This method does yield an improved slideability, but again it affords no improvements in corrosion resistance or paint adherence.

The present invention is directed to solving the problems described above for the prior art. In specific terms, the present invention introduces a composition and method for treating the surface of aluminiferous metal which are able to provide the surface of aluminiferous metal with an excellent corrosion resistance and paint adherence. When applied in particular to Dl aluminum cans, said composition and method impart thereto an excellent slideability in combination with an excellent corrosion resistance and paint adherence.

It has been found that the problems described above for the prior art can be solved through the application of a specific type of surface treatment bath that is prepared using a surface treatment composition containing specific phosphate ions, condensed phosphate ions, and water-soluble polymers with a specific structure. It was found that the application of this surface treatment bath to the surface of aluminiferous metal will form thereon a very corrosion-resistant and highly paint-adherent resin-containing coating. It was also found that application of said bath to Dl aluminum cans forms thereon a resin-containing coating that exhibits an improved slideability in addition to an excellent corrosion resistance and paint adherence. The invention was achieved based on these discoveries.

A composition according to the present invention for treating the surface of aluminiferous metal characteristically comprises, preferably consists essentially of, or more preferably consists of, water and, in parts by weight:
(A) from 1 to 30 parts of phosphate ions;
(B) from 0.1 to 10 parts of condensed phosphate ions; and
(C) from 0.1 to 20 parts of one or more water-soluble polymer(s) conforming with the following general formula (I) in which:
   (i) each of X¹ and X², independently of each other and also from one unit of the polymer [which is defined as any part of the polymer that conforms with the general formula (I) above except that the brackets and the subscript n are omitted] to another unit of the polymer, represents an hydrogen atom, a C₁ to C₅ alkyl group, or a C₁ to C₅ hydroalkyl group;
   (ii) each of Y¹ and Y², independently of each other and also from one unit of the polymer [as defined above] to another, represents an hydrogen atom or a moiety Z that conforms to one or other of the following general formulae: [wherein each of R¹, R², R³, R⁴ and R⁵, independently of each other, represents a C₁ to C₁₀ alkyl group or a C₁ to C₁₀ hydroxyalkyl group];
   (iii) the moiety Z bonded to any single phenyl ring in the polymer molecule may be identical to or may differ from the moiety Z bonded to any other phenyl ring in the polymer molecule;
   (iv) the average value for the number of Z moieties substituted on each phenyl ring in the polymer molecule is in the range of from 0.2 to 1.0;
   (v) n is an integer with a value in the range of from 2 to 50; and
   (vi) each polymer molecule of general formula I contains at least one Z moiety.

'n' is referred to hereinafter as "the average degree of polymerization" and has a value from 2 to 50. Each polymer molecule (I) must contain at least one Z moiety-substituted phenyl ring. This average value for the number of Z moieties substituted on each phenyl ring in the polymer molecules of total component (C) is hereinafter referred to as the average value for Z moiety substitution.

Compositions according to the invention as described above may be either working compositions, suitable for directly treating aluminiferous metal substrates, or they may be concentrate compositions, which are useful for preparing working compositions, usually by dilution of the concentrate compositions with water, and optionally, adjustment of the pH of the resulting working composition.

A method according to the present invention for treating the surface of aluminiferous metal characteristically comprises contacting the surface of aluminiferous metal with a surface treatment bath containing the above-described surface treatment composition according to the present invention, then rinsing the treated surface with water, and subsequently drying the surface by heating. Independently, in a method according to the present invention, the bath preferably has a pH value of 6.5 or less, preferably 2.0 to 6.5, the total time of contacting the metal to be treated preferably is from 5 to 60 seconds, and the temperature during its contact with the aluminiferous metal being treated preferably is from 30°C to 65°C. The reactivity of the bath may be insufficient below 30°C, preventing the formation of a good-quality film. While a good-quality coating is formed at temperatures above 65°C, the higher energy costs for heating make such temperatures economically undesirable. Coating formation may be inadequate and a highly corrosion-resistant coating may not be produced when the immersion time is less than 5 seconds. Long immersion times in excess of 60 seconds usually produce no additional improvements in performance and are disfavored because of their added expense.

Therefore a preferred process according to the invention comprises the steps of:
(I) contacting the surface of the aluminiferous metal for a period of from 5 to 60 seconds at a temperature in the range of from 30°C to 65°C with an aqueous liquid composition according to the invention;
(II) after completion of step (I), separating the surface of the aluminiferous metal from contact with the composition, and rinsing the surface with water; and (III) drying the raised surface of the aluminiferous metal emergent from step II by heating.

The surface treatment method according to the present invention may be implemented by immersing the aluminiferous metal, preferably for 5 to 60 seconds, in the above described surface treatment bath. The surface treatment method according to the present invention may also be implemented by spraying the above-described surface treatment bath onto the surface of the aluminiferous metal, preferably at least twice, and preferably with a nonspray interval of from 2 to 5 seconds between each period of continuous spraying and the next period of continuous spraying if there is one. The occurrence of the pH increase in the vicinity of the interface with the surface, which is required for proper coating formation, is less reliable when spray treatment is carried out by continuously spraying the bath, and in some cases a satisfactory film formation will not occur. It is for this reason that use of an intermittent spray is preferred. The total of the spray and nonspray interval time periods preferably is from 5 to 60 seconds. The reaction may be inadequate and a highly corrosion-resistant coating may not be produced when the total contact time is less than 5 seconds. Lengthy total contact times in excess of 60 seconds usually produce no additional improvements in performance and are more expensive.

A surface treatment composition according to the present invention is an acidic aqueous solution whose essential ingredients are phosphate ion, condensed phosphate ion, and water-soluble polymer with the above-specified chemical structure.

Phosphoric acid (H₃PO₄), sodium phosphate (Na₃PO₄), and the like can be used as the source of the phosphate ion in the surface treatment composition according to the present invention. The phosphate ion content in the above-described formulation ranges from 1 to 30 parts by weight (hereinafter often abbreviated "pbw"), while the preferred range is from 1 to 5 pbw. Reaction between the surface treatment bath and the metal surface will be insufficient and film formation often will be inadequate when the phosphate ions content in the above-described formulation is less than 1 pbw. While a good-quality film is formed with more than 30 pbw of phosphate ions, the high cost of the resulting treatment bath makes such levels economically undesirable.

The condensed phosphate ions used in the present invention conform to the general chemical formula H_{(p+1-q)}PₚO₍₃ₚ₊₁₎^{-q}, where p represents a positive integer that is 2 or greater and q represents a positive integer that is from 1 to (p+1); examples are pyrophosphate ions, tripolyphosphate ions, tetrapolyphosphate ions, and the like. Either the condensed phosphoric acid or its neutral or acid salt can be used as the condensed phosphate ion source for the surface treatment composition according to the present invention. For example, any of pyrophosphoric acid (H₄P₂O₇), disodium diacidpyrophosphate (Na₂H₂P₂O₇), trisodium acidpyrophosphate (Na₃HP₂O₇), and tetrasodium pyrophosphate (Na₄P₂O₇), can be used as the source of the pyrophosphate ions. The condensed phosphate ions content in the above-described formulation for the surface treatment composition according to the present invention, measured as its stoichiometric equivalent of completely ionized condensed phosphate anions conforming to the formula PₚO₍₃ₚ₊₁₎^{-(p+2)}, where p and q have the same meanings as above, ranges from 0.1 to 10 pbw, while the preferred range is from 0.5 to 3.0 pbw. Surface treatment baths prepared using less than 0.1 pbw condensed phosphate ion in the above-described formulation usually have only a weak etching activity and provide inadequate film formation. On the other hand, at more than 10 pbw the etching activity generated by the resulting surface treatment bath is too strong, so that the film-forming reactions are inhibited.

Polymer according to formula (I) with n less than 2 yields only an insufficient improvement in the corrosion resistance of the resulting surface coating. The stability of the corresponding surface treatment composition and surface treatment bath is sometimes inadequate and practical problems often ensue in the case of polymer (I) with n greater than 50.

The presence of 6 or more carbons in the alkyl and hydroxyalkyl groups represented by X¹ and X² in formula (I) causes the resulting polymer molecule to be bulky and produces steric hindrance. This usually interferes with the formation of the fine, dense coatings that exhibit excellent corrosion resistance.

Polymer (I) contains the Z moiety as a substituent, and the average value for Z moiety substitution for each phenyl ring in the polymer molecule must range from 0.2 to 1.0. As an example, in a polymer with n = 10 that has 20 phenyl rings, if only 10 of these 20 phenyl rings are substituted by one Z moiety each, the average value for Z moiety substitution for this polymer is then calculated as follows: (1 x 10)/ 20 = 0.5.

The polymer usually is insufficiently water soluble when the average value for Z moiety substitution is below 0.2; this results in an insufficiently stable surface treatment concentrate and/or surface treatment bath. When, on the other hand, the average value for Z moiety substitution exceeds 1.0 (substitution of a phenyl ring by 2 or more moieties Z), the resulting polymer becomes so soluble in water that formation of an adequately protective surface film is impeded.

The alkyl and hydroxyalkyl moieties encompassed by R¹, R², R³, R⁴, and R⁵ in formulas (II) and (III) should contain from 1 to 10 carbon atoms each. The polymer molecule becomes bulky when this number of carbons exceeds 10; this results in a coarse coating and thereby in an insufficient improvement in the corrosion resistance.

The content of water-soluble polymer (I) in the above-described formulation for the surface treatment composition according to the present invention ranges from 0.1 to 20 pbw, while the range from 0.5 to 5 pbw is preferred. The formation of a coating on the metal surface by the corresponding surface treatment bath often becomes quite problematic when the content of the water-soluble polymer in the above-described formulation is below 0.1 pbw. Values above 20 pbw are economically undesirable due to the increased cost of the surface treatment composition and surface treatment method.

The pH of the surface treatment composition according to the present invention is not narrowly restricted, but adjustment of the pH to values no greater than 6.5, more preferably also not less than 2.0, is generally preferred.

The method according to the present invention is implemented by the preparation of a working surface treatment bath using the above-described surface treatment composition (generally by dilution of a concentrate with water). The pH of the working surface treatment bath at this point is adjusted if necessary to values no greater than 6.5 and preferably to 2.0 to 6.5.

The polymer conforming to formula (I) in the surface treatment bath has a pronounced tendency to deposit or precipitate at a surface treatment bath pH above 6.5; this results in an unsatisfactory stability and service life for the treatment bath. When the pH is below 2.0, the surface treatment bath may etch the metal surface too severely, which can impair formation of the surface coating. The pH of the surface treatment bath may be adjusted using an acid, e.g., phosphoric acid, nitric acid, hydrochloric acid, and the like, or by using alkali, e.g., 'sodium hydroxide, sodium carbonate, ammonium hydroxide, and the like. Hydrofluoric acid may be used to adjust the pH when waste water treatment presents no problems.

When the aluminum ions eluted from the aluminiferous metal being treated according to the invention mixes into the surface treatment bath, a precipitate may be produced in some cases due to the formation of a complex between polymer (I) and the aluminum ions. An aluminum sequestrant is preferably added to the treatment bath in such cases. Suitable as said aluminum sequestrant are, for example, ethylene diamine tetraacetic acid, Cy-DTA, triethanolamine, gluconic acid, heptogluconic acid, oxalic acid, tartaric acid, malic acid, and organophosphonic acids, but the particular sequestrant selection is not critical. Hydrofluoric acid may be used as the sequestrant when it presents no problems for waste water treatment.

A process according to the present invention preferably is performed by contacting the surface of aluminiferous metal with a surface treatment bath - prepared as described above - at 30° C to 65° C for a total of 5 to 60 seconds. The process then continues with a water rinse of the film formed on the metal surface and drying by heating.

Problems with the coating can occur due to foaming of the surface treatment bath when a spray treatment is used. The generation of foam and the intensity of foaming strongly depend on the type of spray equipment and the spraying conditions, and a defoamer is preferably added to the surface treatment bath when a foaming problem cannot be satisfactorily resolved by changes to the spray equipment andlor conditions. Such factors as the type and dispensing level of the defoamer are not critical, provided that they do not impair the paint adherence of the resulting coating.

A preferred method of preparation of a surface treatment composition according to the present invention will now be briefly summarized. To prepare the surface treatment composition, the phosphate ions and condensed phosphate ions are first made up in the above-described proportions and dissolved with thorough stirring in the required amount of water according to the preceding specifications. When the pH of the resulting solution exceeds 7, it is adjusted to less than or equal to 7 using a suitable acid as described above. The water-soluble resin specified by the invention is then added while stirring and completely dissolved, and the pH is adjusted to less than or equal to 6.5 as described above.

The coating formed on the surface of aluminiferous metal will now also be briefly discussed. The coating formed by the surface treatment bath according to the present invention is an organic-inorganic composite coating whose main components are phosphate salt and polymer (I). Etching of the metal surface by the phosphate ions and condensed phosphate ions causes a local increase in pH to occur at the interface; this results in deposition of phosphate salt on the metal surface. In addition, the chelating activity of the amino group in polymer (I) may result in the formation of a coordination compound with the fresh substrate surface exposed by etching. The presence of condensed phosphate ions in the surface treatment bath is believed to promote formation of the polymer-metal coordination compound and thereby make possible stable formation of the organic-inorganic composite coating on the surface over a broad pH range.

An additional polymerization of the polymer present on the surface can be induced by heating the surface coating after its formation. In specific cases where an elevated corrosion resistance is required, the coating is preferably heated in order to produce a higher molecular weight for the polymer on the surface. Suitable heating conditions for this purpose are at least 1 minute and at least 200° C.

Aluminiferous metal substrates that may be subjected to the method according to the present invention comprise, for example, the sheet, bar, tube, wire, and like shapes, of aluminum and its alloys, e.g., aluminum-manganese alloys, aluminum-magnesium alloys, aluminum-silicon alloys, and the like. There are absolutely no limitations on the dimensions or shape of the aluminiferous metal.

The polymer composition according to the present invention may contain a preservative or antimold agent. These function to inhibit putrefaction or mold growth when the surface treatment bath is used or stored at low temperatures. Hydrogen peroxide is a specific example in this regard.

The following is a short discussion of further details of a process of treating the surface of aluminiferous metal using the surface treatment bath according to the present invention. The process steps outlined below are a preferred example of application of the surface treatment bath according to the present invention.
(1) Surface cleaning: degreasing - an acidic, alkaline, or solvent-based degreaser may be used.
(2) Water rinse
(3) Film-forming treatment (surface treatment method according to the present invention)
(4) Water rinse
(5) Rinse with de-ionized water
(6) Drying

The invention is illustrated in greater detail below through working examples, and its benefits may be further appreciated by contrast with the comparison examples. The individual surface treatment bath components and surface treatment methods are respectively described in the working and comparative examples.

### Examples

### Evaluation Methods

### (1) Corrosion resistance

The corrosion resistance of the unpainted parts of the Dl aluminum cans (resistance to blackening by boiling water) was evaluated based on the degree of discoloration (blackening) after immersion of treated Dl aluminum cans in boiling tap water for 30 minutes. The results of this test are reported on the following scale:
- + :: no blackening
- x :: partial blackening
- xx :: blackening over entire surface

### (2) Paint adherence

The paint adherence was tested as follows. The surface of the treated can was coated to a paint film thickness of 5 to 7 micrometers with an epoxy-urea can paint. This was followed by baking for 4 minutes at 215° C. A 5 millimeter (hereinafter usually abbreviated "mm") x 150 mm strip was then cut from the painted can and hot-press bonded with polyamide film to give a test specimen. The test specimen thus prepared was subjected to a 180° peel test, during which the peel strength was measured. Higher peel strength values in this test are indicative of a better paint adherence, and peel strength values equal to or greater than 4.0 kilograms-force per 5 millimeters of width (hereinafter usually abbreviated as "kgf/5mm") are generally regarded as excellent from the standpoint of practical applications.

### (3) Slideability

The slideability was evaluated by measuring the static friction coefficient on the outside surface of the can. Lower values for the static friction coefficient are indicative of a better siideability, and values less than or equal to 1.0 are generally regarded as excellent.

### Example 1

DI aluminum cans fabricated by the DI processing of A3004 aluminum alloy sheet were cleaned by first degreasing with a 60-second spray at 75° C of an 8 % aqueous solution of PALKLIN™ 500 acidic degreaser manufactured by Nihon Parkerizing Company, Limited and then rinsing with water. The cleaned surface was subsequently sprayed with Surface Treatment Bath 1 (composition given below) heated to 60° C. The spray treatment consisted of 3 sprays of 5 seconds each separated by 5 second intervals for a total of 25 seconds. This was followed in order by rinsing with tap water, spraying for 10 seconds with de-ionized water (with a resistivity of at least 3,000,000 ohm-cm), and drying in a hot-air drying oven at 180° C for 2 minutes.

| Surface Treatment Bath 1 | | |
|---|---|---|
| 75 % Aqueous phosphoric acid (H₃PO₄) | 10.0 g/L | (PO₄⁻³ ions: 7.2 g/L) |
| Sodium pyrophosphate (Na₄P₂O₇• 10H₂O) | 3.0 g/L | (P₂O₇⁻⁴ ions: 1.2 g/L) |
| Water-Soluble Polymer 1 | 2.0 g/L | (solids) |
| pH: 4.0 (adjusted with sodium hydroxide) | | |
| Balance: water | | |

For Water-Soluble Polymer 1, n = 5, X¹ and X² = hydrogen, Z = -CH₂N(CH₃)₂ in formula (I), and the average value for Z moiety substitution = 0.25.

### Example 2

The Dl aluminum cans were cleaned according to the procedure described in Example 1 and then immersed for 20 seconds in Surface Treatment Bath 2 (composition given below) heated to 60° C. This treatment was followed by rinsing with water and drying according to the procedure described in Example 1.

| Surface Treatment Bath 2 | | |
|---|---|---|
| 75 % Aqueous phosphoric acid (H₃PO₄) | 10.0 g/L | (PO₄⁻³ ions: 7.2 g/L) |
| sodium pyrophosphate (Na₄P₂O·10H₂O) | 3.0 g/L | (P₂O₇⁻⁴ ions: 1.2 g/L) |
| Water-Soluble Polymer 1 | 0.4 g/L | (solids) |
| pH: 3.0 (adjusted with sodium carbonate) | | |
| Balance: water | | |

Water-Soluble Polymer 1 was the same as described in Example 1.

### Example 3

The Dl aluminum cans were cleaned according to the procedure described in Example 1 and then immersed for 60 seconds in Surface Treatment Bath 3 (composition given below) heated to 35° C. This treatment was followed by rinsing with water and drying according to the procedure described in Example 1.

| Surface Treatment Bath 3 | | |
|---|---|---|
| 75 % Aqueous phosphoric acid (H₃PO₄) | 20.0 g/L | (PO₄⁻³ ions: 14.4 g/L) |
| Sodium pyrophosphate (Na₄P₂O₇• 10H₂O) | 6.0 g/L | (P₂O₇⁻⁴ ions: 2.4 g/L) |
| Water-Soluble Polymer 1 | 8.0 g/L | (solids) |
| pH: 6.0 (adjusted with sodium hydroxide) | | |
| Balance: water | | |

Water-Soluble Polymer 1 was the same as described in Example 1.

### Example 4

The Dl aluminum cans were cleaned according to the procedure described in Example 1 and then sprayed with Surface Treatment Bath 4 (composition given below) heated to 65° C. The spray treatment consisted of 3 sprays (6 seconds each) separated by intervals of 2 seconds (total of 22 seconds). This treatment was followed by rinsing with water and drying according to the procedure described in Example 1.

| Surface Treatment Bath 4 | | |
|---|---|---|
| 75 % Aqueous phosphoric acid (H₃PO₄) | 1.5 g/L | (PO₄⁻³ ions: 1.1 g/L) |
| Sodium pyrophosphate (Na₄P₂O₇•10H₂O) | 5.0 g/L | (P₂O₇⁻⁴ ions: 2.0 g/L) |
| Water-Soluble Polymer 1 | 4.0 g/L | (solids) |
| pH: 2.5 (adjusted with nitric acid) | | |
| Balance: water | | |

Water-Soluble Polymer 1 was the same as described in Example 1.

### Example 5

The Dl aluminum cans were cleaned according to the procedure described in Example 1 and then immersed for 30 seconds in Surface Treatment Bath 5 (composition given below) heated to 60° C. This treatment was followed by rinsing with water and drying according to the procedure described in Example 1.

| Surface Treatment Bath 5 | | |
|---|---|---|
| 75 % Aqueous phosphoric acid (H₃PO₄) | 30.0 g/L | (PO₄⁻³ ions: 21.6 g/L) |
| Sodium tripolyphosphate (Na₅P₃O₁₀) | 1.2 g/L | (P₃O₁₀⁻⁵ ions: 0.8 g/L) |
| Water-Soluble Polymer 1 | 2.0 g/L | (solids) |
| pH: 3.5 (adjusted with sodium hydroxide) | | |
| Balance: water | | |

Water-Soluble Polymer 1 was the same as described in Example 1.

### Example 6

The Dl aluminum cans were cleaned according to the procedure described in Example 1 and then sprayed with Surface Treatment Bath 6 (composition given below) heated to 60° C. The spray treatment consisted of 2 sprays of 5 seconds each separated by an interval of 5 seconds for a total of 15 seconds). This treatment was followed by rinsing with water and drying according to the procedure described in Example 1.

| Surface Treatment Bath 6 | | |
|---|---|---|
| 75 % Aqueous phosphoric acid (H₃PO₄) | 10.0 g/L | (PO₄⁻³ ions: 7.2 g/L) |
| Sodium pyrophosphate (Na₄P₂O₇• 10 H₂O) | 3.0 g/L | (P₂O₇⁻⁴ ions: 1.2 g/L) |
| Water-Soluble Polymer 2 | 2.0 g/L | (solids) |
| pH: 5.0 (adjusted with sodium hydroxide) | | |
| Balance: water | | |

For Water-Soluble Polymer 2, in formula (I), n = 5, X¹ and X² = -C₂H₅, and Z = -CH₂N(CH₂CH₂OH)₂, and the average value for Z moiety substitution = 1.0.

### Example 7

The Dl aluminum cans were cleaned according to the procedure described in Example 1 and then immersed for 30 seconds in Surface Treatment Bath 7 (composition given below) heated to 60° C. This treatment was followed by rinsing with water and drying according to the procedure described in Example 1.

| Surface Treatment Bath 7 | | |
|---|---|---|
| 75 % Aqueous phosphoric acid (H₃PO₄) | 10.0 g/L | (PO₄⁻³ ions: 7.2 g/L) |
| Sodium pyrophosphate (Na₄P₂O₇• 10H₂O) | 3.0 g/L | (P₂O₇⁻⁴ ions: 1.2 g/L) |
| Water-Soluble Polymer 3 | 2.0 g/L | (solids) |
| pH: 4.0 (adjusted with sodium hydroxide) | | |
| Balance: water | | |

For Water-Soluble Polymer 3, in formula (I), n = 2, X¹ and X² = -C₂H₅, and Z = -CH₂N(CH₂CH₂CH₂OH)₂, and the average value for Z moiety substitution = 0.6.

### Comparative Example 1

The Dl aluminum cans were cleaned according to the procedure described in Example 1 and then sprayed with Surface Treatment Bath 8 (composition given below) heated to 60° C. The spray treatment consisted of 5 sprays of 4 seconds each separated by intervals of 5 seconds each, for a total of 40 seconds. This treatment was followed by rinsing with water and drying according to the procedure described in Example 1.

| Surface Treatment Bath 8 | | |
|---|---|---|
| 75 % Aqueous phosphoric acid (H₃PO₄) | 10.0 g/L | (PO₄⁻³ ions: 7.2 g/L) |
| Water-Soluble Polymer 1 | 2.0 g/L | (solids) |
| pH: 3.0 (adjusted with sodium carbonate) | | |
| Balance: water | | |

Water-Soluble Polymer 1 was the same as described in Example 1.

### Comparative Example 2

The DI aluminum cans were cleaned according to the procedure described in Example 1 and then immersed for 30 seconds in Surface Treatment Bath 9 (composition given below) heated to 60° C. This treatment was followed by rinsing with water and drying according to the procedure described in Example 1.

| Surface Treatment Bath 9 | | |
|---|---|---|
| 75 % Aqueous phosphoric acid (H₃PO₄) | 1.0 g/L | (PO₄⁻³ ions: 0.72 g/L) |
| Water-Soluble Polymer 1 | 2.0 g/L | (solids) |
| pH: 7.0 (adjusted with sodium hydroxide) | | |
| Balance: water | | |

Water-Soluble Polymer 1 was the same as described in Example 1.

### Comparative Example 3

The Dl aluminum cans were cleaned according to the procedure described in Example 1 and then immersed for 5 seconds in Surface Treatment Bath 10 (composition given below) heated to 60° C. This treatment was followed by rinsing with water and drying according to the procedure described in Example 1.

| Surface Treatment Bath 10 | | |
|---|---|---|
| 75 % Aqueous phosphoric acid (H₃PO₄) | 10.0 g/L | (PO₄⁻³ ions: 7.2 g/L) |
| Sodium pyrophosphate (Na₄P₂O₇ • 10H₂O) | 1.0 g/L | (P₂O₇⁻⁴ ions: 0.4 g/L) |
| Water-Soluble Polymer 1 | 0.05 g/L | (solids) |
| pH: 4.0 (adjusted with sodium carbonate) | | |
| Balance: water | | |

Water-Soluble Polymer 1 was the same as described in Example 1.

### Comparative Example 4

The Dl aluminum cans were cleaned according to the procedure described in Example 1 and then immersed for 20 seconds in Surface Treatment Bath 11 (composition given below) heated to 60° C. This treatment was followed by rinsing with water and drying according to the procedure described in Example 1.

| Surface Treatment Bath 11 | | |
|---|---|---|
| 95 % Aqueous sulfuric acid (H₂SO₄) | 2.0 g/L | (SO₄⁻² ions: 1.9 g/L) |
| Sodium pyrophosphate (Na₄P₂O₇ • 10H₂O) | 1.0 g/L | (P₂O₇ ion: 0.4 g/L) |
| Water-Soluble Polymer 1 | 0.05 g/L | (solids) |
| pH: 3.5 (adjusted with sodium carbonate) | | |

Water-Soluble Polymer 1 was the same as described in Example 1.

### Comparative Example 5

The Dl aluminum cans were cleaned according to the procedure described in Example 1 and then immersed for 30 seconds in Surface Treatment Bath 12 (composition given below) heated to 60° C. This treatment was followed by rinsing with water and drying according to the procedure described in Example 1.

| Surface Treatment Bath 12 | | |
|---|---|---|
| 75 % Aqueous phosphoric acid (H₃PO₄) | 1.0 g/L | (PO₄⁻³ ions: 0.72 g/L) |
| Sodium pyrophosphate (Na₄P₂O₇•10 H₂O) | 1.0 g/L | (P₂O₇⁻⁴ ions: 0.4 g/L) |
| Water-Soluble Polymer 4 | 2.0 g/L | (solids) |
| pH: 4.0 (adjusted with sodium hydroxide) | | |
| Balance: water | | |

For Water-Soluble Polymer 4, in formula (I), n = 5, X¹ and X² = -C₂H₅, and Z = -CH₂SO₃H, and the average value for -CH₂SO₃H substitution = 0.6.

### Comparative Example 6

The DI aluminum cans were cleaned according to the procedure described in Example 1 and then immersed for 30 seconds in Surface Treatment Bath 13 (composition given below) heated to 60° C. This treatment was followed by rinsing with water and drying according to the procedure described in Example 1.

| Surface Treatment Bath 13 (surface treatment bath described in Japanese Patent Application Laid Open [Kokai or Unexamined] Number Hei 4-66671) | | |
|---|---|---|
| 75 % Aqueous phosphoric acid (H₃PO₄) | 1.0 g/L | (PO₄⁻³ ions: 0.72 g/L) |
| Sodium pyrophosphate (Na₄P₂O₇• 10 H₂O) | 1.0 g/L | (P₂O₇⁻⁴ ions: 0.4 g/L) |
| Water-Soluble Polymer 5 | 2.0 g/L | (solids) |
| pH: 4.0 (adjusted with sodium hydroxide) | | |
| Balance: water | | |

Water-Soluble Polymer 5 had the following formula (IV):

### Comparative Example 7

The Dl aluminum cans were cleaned according to the procedure described in Example 1 and then immersed for 30 seconds in Surface Treatment Bath 14 (composition given below) heated to 60° C. This treatment was followed by rinsing with water and drying according to the procedure described in Example 1.

| Surface Treatment Bath 14 | | |
|---|---|---|
| 75 % Aqueous phosphoric acid (H₃PO₄) | 1.0 g/L | (PO₄⁻³ ions: 0.72 g/L) |
| Sodium pyrophosphate (Na₄P₂O₇• 10 H₂O) | 1.0 g/L | (P₂O₇⁻⁴ ions: 0.4 g/L) |
| Water-Soluble Polymer 6 | 2.0 g/L | (solids) |
| pH: 4.0 (adjusted with sodium hydroxide) | | |
| Balance: water | | |

Water-Soluble Polymer 6 had the following formula (V) (resin described in Japanese Patent Application Laid Open [Kokai or Unexamined] Number Hei 2-608):

### Comparative Example 8

The Dl aluminum cans were cleaned according to the procedure described in Example 1 and then sprayed with the 2% aqueous solution of a non-chromate surface treatment agent (brand name ALO DINE® 404 non-chromate surface treatment agent, manufactured by Nihon Parkerizing Company, Limited, heated to 40° C. This spray treatment consisted of 3 sprays of 5 seconds each separated by 5 second intervals for a total of 25 seconds. This treatment was followed by rinsing with water and drying according to the procedure described in Example 1.

The evaluation results for Examples 1 to 7 and Comparative Examples 1 to 8 are reported in Table 1.

**Table 1.**

| Results of the Evaluations | | | |
|---|---|---|---|
| **Example or Comparison Example Number** | **Blackening Resistance** | **Peel Strength, kgf/5mm** | **Coefficient of Static Friction** |
| Example 1 | + | 4.0 | 0.9 |
| Example 2 | + | 4.0 | 0.9 |
| Example 3 | + | 4.0 | 0.9 |
| Example 4 | + | 4.0 | 0.9 |
| Example 5 | + | 4.0 | 0.9 |
| Example 6 | + | 4.0 | 0.9 |
| Example 7 | + | 4.0 | 0.9 |
| Comparative Example 1 | x | 2.0 | 1.3 |
| Comparative Example 2 | x x | 1.5 | 1.5 |
| Comparative Example 3 | x x | 2.0 | 1.5 |
| Comparative Example 4 | x x | 1.5 | 1.5 |
| Comparative Example 5 | x x | 1.5 | 1.6 |
| Comparative Example 6 | + | 2.0 | 1.1 |
| Comparative Example 7 | x x | 1.5 | 1.6 |
| Comparative Example 8 | + | 4.0 | 1.6 |

As the results in Table 1 make clear, Examples 1 to 7, which used surface treatment compositions and surface treatment methods according to the present invention, yielded surface-treated metals with an excellent blackening resistance, excellent adherence, and excellent slideability. In contrast to this, satisfactory values could not be simultaneously obtained for all these properties (corrosion resistance, paint adherence, and slideability) in the case of the surface-treated metals afforded by surface treatment baths outside the scope of the present invention (Comparative Examples 1 to 8).

### Benefits of the Invention

As the preceding description has made clear, the surface treatment composition and surface treatment method according to the present invention can produce very corrosion-resistant and highly paint-adherent conversion coatings on the surface of aluminiferous metals prior to the painting thereof. In particular, application of the surface treatment composition according to the present invention to the treatment of Dl aluminum cans results in the formation on the surface of Dl aluminum cans prior to its painting or printing of a very corrosion-resistant and highly paint-adherent film that also provides the excellent slideability required for smooth conveyor transport of the can. Since the surface treatment composition according to the present invention and the surface treatment bath used in the invention method do not contain chromium or fluorine, they have the excellent advantage of reducing the load on waste water treatment.

## Claims

1. An aqueous liquid composition for treating the surface of aluminiferous metals, either as such or after dilution with additional water, said composition comprising water and:
**(A)** from 1 to 30 pbw of phosphate ions;
**(B)** from 0.1 to 10 pbw of condensed phosphate ions; and
**(C)** from 0.1 to 20 pbw of one or more water-soluble polymer(s) conforming with the following general formula: in which:
**(i)** each of X¹ and X², independently of each other and also from one unit of the polymer [which is defined as any part of the polymer that conforms with the general formula (I) above except that the brackets and the subscript n are omitted] to another unit of the polymer, represents an hydrogen atom, a C₁ to C₅ alkyl group, or a C₁ to C₅ hydroxyalkyl group;
**(ii)** each of Y¹ and Y², independently of each other and also from one unit of the polymer [as defined above] to another, represents an hydrogen atom or a moiety Z that conforms to one or other of the following general formulae: [wherein each of R¹, R², R³, R⁴ and R⁵, independently of each other, represents a C₁ to C₁₀ alkyl group or a C₁ to C₁₀ hydroxyalkyl group];
**(iii)** the moiety Z bonded to any single phenyl ring in the polymer molecule may be identical to or may differ from the moiety Z bonded to any other phenyl ring in the polymer molecule;
**(iv)** the average value for the number of Z moieties substituted on each phenyl ring in the polymer molecule is in the range of from 0.2 to 1.0;
**(v)** n is an integer with a value in the range of from 2 to 50; and
**(vi)** each polymer molecule of general formula I contains at least one Z moiety.

2. A composition as claimed in claim 1, comprising from 1 to 5 pbw of the phosphate ions, from 0.5 to 3 pbw of the condensed phosphate ions, and from 0.5 to 5 pbw of the water-soluble polymer(s) conforming with general formula (I).

3. A composition as claimed in claim 1 or claim 2, having a pH value not greater than 6.5 and comprising from 1 to 30 g/L of the phosphate ions, from 0.1 to 10 g/L of the condensed phosphate ions, and from 0.1 to 20 g/L of the water-soluble polymer(s) conforming with formula (I).

4. A composition as claimed in claim 3, having a pH value in the range of from 2.0 to 6.5.

5. A composition as claimed in any of the preceding claims, which also includes an aluminium sequestrant.

6. A process for treating a surface of aluminiferous metal, said process comprising steps of:
(I) contacting the surface of the aluminiferous metal for a period of from 5 to 60 seconds at a temperature in the range of from 30°C to 65°C with an aqueous liquid composition as claimed in any of the preceding claims;
(II) after completion of step (I), separating the surface of the aluminiferous metal from contact with the composition, and rinsing the surface with water; and
(III) drying the raised surface of the aluminiferous metal emergent from step II by heating.

7. A process as claimed in claimed 6, wherein step (I) is accomplished by immersing the aluminiferous metal surface in the composition.

8. A process as claimed in claim 6, wherein step (I) is accomplished by spraying the composition onto the aluminiferous metal surface.

9. A process as claimed in claim 8, wherein:
the aluminiferous metal surface is sprayed at least twice; the periods of spraying contact are interrupted by non-spraying intervals having a duration in the range of from 2 to 5 seconds; and
the total time between completing the first spraying and ending the last spraying is in the range of from 5 to 60 seconds.

10. A process as claimed in any of claims 6 to 9, which also includes the subsequent step of inducing additional polymerization of the polymer present on the treated surface by heating thereof for a period of at least 1 minute to a temperature of at least 200°C.

## Patentansprüche

1. Wäßrige, flüssige Zusammensetzung, entweder als solche oder nach dem Verdünnen mit zusätzlichem Wasser, zur Behandlung der Oberfläche aluminiumhaltiger Metalle, wobei die Zusammensetzung Wasser und
(A) 1 bis 30 Gewichtsteile Phosphationen;
(B) 0,1 bis 10 Gewichtsteile kondensierte Phosphationen und
(C) 0,1 bis 20 Gewichtsteile eines oder mehrerer wasserlöslicher Polymere gemäß der folgenden allgemeinen Formel: umfaßt, worin
(i) jedes von X¹ und X² unabhängig voneinander und auch von einer Einheit des Polymers [welche als jeder Teil des Polymers definiert ist, der mit der allgemeinen Formel (I) oben übereinstimmt, außer daß die Klammern und der tiefgestellte Index n weggelassen sind] zu einer anderen Einheit des Polymers ein Wasserstoffatom, eine C₁- bis-C₅-Alkylgruppe oder eine C₁- bis C₅-Hydroxyalkylgruppe darstellt;
(ii) jedes von Y¹ und Y² unabhängig voneinander und auch von einer Einheit des Polymers [wie oben definiert] zu einer anderen ein Wasserstoffatom oder einen Rest Z darstellt, der mit einer oder einer anderen der folgenden allgemeinen Formeln: übereinstimmt [worin jedes von R¹, R², R³, R⁴ und R⁵ unabhängig voneinander eine C₁- bis C₁₀-Alkylgruppe oder eine C₁- bis C₁₀-Hydroxyalkylgruppe darstellt] ;
(iii) der Rest Z, der an jeden einzelnen Phenylring in dem Polymermolekül gebunden ist, identisch oder von dem Rest Z unterschieden sein kann, der an jeden anderen Phenylring in dem Polymermolekül gebunden ist;
(iv) der durchschnittliche Wert für die Anzahl der Z-Reste, die an jedem Phenylring in dem Polymermolekül substituiert sind, im Bereich von 0,2 bis 1,0 liegt;
(v) jedes Polymermolekül der allgemeinen Formel I wenigstens einen Z-Rest enthält.

2. Zusammensetzung gemäß Anspruch 1, umfassend 1 bis 5 Gewichtsteile der Phosphationen, 0,5 bis 3 Gewichtsteile der kondensierten Phosphationen und 0,5 bis 5 Gewichtsteile des wasserlöslichen Polymers (der wasserlöslichen Polymere) gemäß der allgemeinen Formel I.

3. Zusammensetzung gemäß Anspruch 1 oder Anspruch 2, die eine pH-Wert von nicht größer als 6,5 aufweist und 1 bis 30 g/l der Phosphationen, 0,1 bis 10 g/l der kondensierten Phosphationen und 0,1 bis 20 g/l des wasserlöslichen Polymers (der wasserlöslichen Polymere) gemäß der allgemeinen Formel I umfaßt.

4. Zusammensetzung gemäß Anspruch 3 mit einem pH-Wert im Bereich von 2,0 bis 6,5.

5. Zusammensetzung gemäß irgendeinem der vorhergehenden Ansprüche, die auch ein Aluminium-Maskierungsmittel einschließt.

6. Verfahren zur Behandlung einer Oberfläche von aluminiumhaltigem Metall, umfassend die Stufen
(I) des In-Kontakt-Bringens des aluminiumhaltigen Metalls während einer Zeitspanne von 5 bis 60 Sekunden bei einer Temperatur im Bereich von 30 °C bis 65 °C mit einer wäßrigen, flüssigen Zusammensetzung gemäß irgendeinem der vorhergehenden Ansprüche;
(II) des Aufhebens des Kontakts zwischen der Oberfläche des aluminiumhaltigen Metalls und der Zusammensetzung nach der Vervollständigung der Stufe (I) und des Spülens der Oberfläche mit Wasser; und
(III) des Trocknens der erhöhten Oberfläche des aluminiumhaltigen Metalls, die sich aus der Stufe II ergibt, durch Erwärmen.

7. Verfahren gemäß Anspruch 6, worin die Stufe (I) durch Eintauchen der aluminiumhaltigen Metalloberfläche in die Zusammensetzung erreicht wird.

8. Verfahren gemäß Anspruch 6, worin die Stufe (I) durch Sprühen der Zusammensetzung auf die Oberfläche des aluminiumhaltigen Metalls erreicht wird.

9. Verfahren gemäß Anspruch 8, worin die Oberfläche des aluminiumhaltigen Metalls wenigstens zweimal besprüht wird; die Sprühkontakt-Perioden durch Nichtsprüh-Intervalle unterbrochen werden, die eine Dauer im Bereich von 2 bis 5 Sekunden haben; und die Gesamtzeit zwischen der Vervollständigung des ersten Sprühens und der Beendigung des letzten Sprühens im Bereich von 5 bis 60 Sekunden liegt.

10. Verfahren gemäß irgendeinem der Ansprüche 6 bis 9, welches auch die nachfolgende Stufe des Herbeiführens einer zusätzlichen Polymerisation des auf der behandelten Oberfläche vorliegenden Polymers durch Erwärmen desselben während einer Zeitspanne von wenigstens 1 Minute auf eine Temperatur von wenigstens 200 °C einschließt.

## Revendications

1. Composition liquide aqueuse pour traiter la surface de métaux contenant de l'aluminium, en l'état ou après dilution avec de l'eau supplémentaire, ladite composition comprenant de l'eau et:
(A) de 1 à 30 parties en masse d'ions phosphate;
(B) de 0,1 à 10 parties en masse d'ions phosphate condensés; et
(C) de 0,1 à 20 parties en masse d'un ou plusieurs polymères hydrosolubles répondant à la formule générale suivante: dans laquelle:
(i) X¹ et X², indépendamment l'un de l'autre et aussi d'une unité du polymère [qui est définie par toute partie du polymère qui répond à la formule générale (I) ci-dessus à ceci près que les crochets et l'indice n sont omis] à une autre unité du polymère, représentent chacun un atome d'hydrogène, un groupe alkyle en C₁ à C₅ ou un groupe hydroxyalkyle en C₁ à C₅;
(ii) Y¹ et Y², indépendamment l'un de l'autre et aussi d'une unité du polymère [comme défini ci-dessus] à une autre, représentent chacun un atome d'hydrogène ou une entité Z qui répond à l'une ou l'autre des formules générales suivantes: [où R¹, R², R³, R⁴ et R⁵, indépendamment les uns des autres, représentent chacun un groupe alkyle en C₁ à C₁₀ ou un groupe hydroxyalkyle en C₁ à C₁₀];
(iii) l'entité Z liée à tout cycle phényle individuel dans la molécule de polymère peut être identique à ou différente de l'entité Z liée à tout autre cycle phényle dans la molécule de polymère;
(iv) la valeur moyenne du nombre d'entités Z comme substituants sur chaque cycle phényle dans la molécule de polymère est dans le domaine de 0,2 à 1,0;
(v) n est un entier ayant une valeur dans le domaine de 2 à 50; et
(vi) chaque molécule de polymère de formule générale I contient au moins une entité Z.

2. Composition selon la revendication 1 comprenant de 1 à 5 parties en masse d'ions phosphate, de 0,5 à 3 parties en masse d'ions phosphate condensés et de 0,5 à 5 parties en masse de polymère(s) hydrosoluble(s) répondant à la formule générale (I).

3. Composition selon la revendication 1 ou la revendication 2 ayant un pH d'au plus 6,5 et comprenant de 1 à 30 g/l d'ions phosphate, de 0,1 à 10 g/l d'ions phosphate condensés et de 0,1 à 20 g/l de polymère(s) hydrosoluble(s) répondant à la formule (I).

4. Composition selon la revendication 3 ayant un pH dans le domaine de 2,0 à 6,5.

5. Composition selon l'une quelconque des revendications précédentes qui comprend aussi un séquestrant de l'aluminium.

6. Procédé pour traiter une surface de métal contenant de l'aluminium, ledit procédé comprenant les étapes de:
(I) mise en contact de la surface du métal contenant de l'aluminium pendant une durée de 5 à 60 secondes à une température dans le domaine de 30°C à 65°C avec une composition liquide aqueuse selon l'une quelconque des revendications précédentes;
(II) après l'achèvement de l'étape (I), séparation de la surface du métal contenant de l'aluminium d'avec la composition, et rinçage de la surface à l'eau; et (III) séchage de la surface relevée du métal contenant de l'aluminium provenant de l'étape II par chauffage.

7. Procédé selon la revendication 6 dans lequel l'étape (I) est accomplie par immersion de la surface du métal contenant de l'aluminium dans la composition.

8. Procédé selon la revendication 6 dans lequel l'étape (I) est accomplie par pulvérisation de la composition sur la surface du métal contenant de l'aluminium.

9. Procédé selon la revendication 8 dans lequel:
la surface du métal contenant de l'aluminium est soumise à la pulvérisation au moins deux fois; les périodes de contact par pulvérisation sont interrompues par des intervalles sans pulvérisation ayant une durée dans le domaine de 2 à 5 secondes; et
la durée totale entre l'accomplissement de la première pulvérisation et la fin de la dernière pulvérisation est dans le domaine de 5 à 60 secondes.

10. Procédé selon l'une quelconque des revendications 6 à 9 qui comprend aussi l'étape subséquente d'induire une polymérisation supplémentaire du polymère présent sur la surface traitée par chauffage de celui-ci pendant une durée d'au moins 1 minute à une température d'au moins 200°C.
